

# UNITED STATES PATENT OFFICE.

MORITZ VON GALLOIS, OF HÖCHST-ON-THE-MAIN, GERMANY, ASSIGNOR TO FARBWERKE, VORM. MEISTER, LUCIUS & BRÜNING, OF HÖCHST-ON-THE-MAIN, GERMANY, A CORPORATION OF GERMANY.

## PROCESS OF PRINTING WITH INDIGO.

No. 808,443.

Specification of Letters Patent.

Patented Dec. 26, 1905.

Application filed April 21, 1904. Serial No. 204,287.

*To all whom it may concern:*

Be it known that I, MORITZ VON GALLOIS, chemist, a citizen of the Empire of Austria-Hungary, residing at Höchst - on - the - Main,

5 Germany, have invented certain new and useful Improvements in Printing Fabrics with Indigo, of which the following is a specification.

By the present invention in printing indigo 10 by the hydrosulfite method strong caustic alkalies are substituted for the alkali salts previously used. This substitution is particularly applicable to printing with the stable hydrosulfite compounds made by combining 15 an aldehyde or derivative or analogue thereof with hydrosulfurous acid or a salt or double salt thereof.

By the present method white fabrics and fabrics dyed with certain other colors, such as 20 alizarine red, may be printed.

### Examples.

#### Indigo-Blue Steam-Printing Color.

25 A { 120 grams of formaldehyde compound of sodium hydrosulfite are dissolved in  
50 grams of water at 40° to 50° centigrade, cooled, and slowly stirred into  
500 grams of alkali thickener.

B { 150 grams of indigo paste of twenty per cent. strength stirred with  
180 grams of alkaline thickener, then cooled, and B stirred into A.

30 1 kilo.

#### Alkaline Thickener.

120 grams of gomme industrielle (E. Bernard & Cie., Mühlhausen i. E.) are dissolved in 430 grams of hot water, and when cold are added slowly to 450 grams of solid caustic soda while stirring continuously.

1 kilo.

35

The bleached cotton (unprepared) or cotton dyed with Turkey red is printed with this indigo blue steam-printing color, well dried, and then steamed in the Mather Platt apparatus for two or three minutes at 90° to 100° centigrade, 40 then well washed, whereupon the indigo white oxidizes to indigo blue. The fabric is then acidified and soaped, if necessary.

Having now described my invention, what I claim is—

45

The improvement in the process of printing fabrics with indigo on white or Turkey red dyed unprepared cotton, which consists in simultaneously applying in the printing color a mixture of indigo and stable double compounds of hydrosulfites with aldehydes and strong caustic alkalies.

In testimony that I claim the foregoing as my invention I have signed my name in presence of two subscribing witnesses.

MORITZ VON GALLOIS.

Witnesses:

ALFRED BRISBOIS,  
JOSEPH FLACH.